

Patented July 1, 1924.

1,499,930

# UNITED STATES PATENT OFFICE.

FREDERIC EUGENE IVES, OF PHILADELPHIA, PENNSYLVANIA.  
PHOTOGRAPHIC PROCESS.

No Drawing.

Application filed October 25, 1923. Serial No. 670,658.

To all whom it may concern:

Be it known that I, FREDERIC EUGENE IVES, a citizen of the United States, residing at Philadelphia, county of Philadelphia, State 5 of Pennsylvania, have invented a new and useful Photographic Process, of which the following is a specification.

My invention has for its main object the conversion by a single bath or process of a 10 photographic silver image in a colloid layer containing also silver bromide, to a pigment blue print and silver bromide.

This I accomplish by immersing the un-fixed silver print in a chemical blue-toning 15 bath which contains in addition to the other necessary ingredients one or more suitable haloids, or halids.

The silver print is made by exposure and development of a gelatine-bromide or other 20 suitable sensitive layer, which may be on either an opaque or a transparent carrier, and after development and washing, but without fixing, and preferably without exposure to actinic light, is immersed for a 25 sufficient period in a bath containing the necessary ingredients. A suitable bath for this purpose consists of:—

|                                |             |
|--------------------------------|-------------|
| Water                          | 20 litres   |
| Oxalic acid                    | 85 grammes  |
| Potassium ferricyanide         | 35 grammes  |
| Sodium chloride                | 85 grammes  |
| Potassium bromide              | 7 grammes   |
| U. S. P. ferric chloride solu. | 20 c. c. s. |

An immersion of ten minutes is usually 35 sufficient to complete the reaction, but a longer immersion is to be recommended. The product is a pigment blue print buried in an even layer of light-sensitive silver bromide, in which another image can be subsequently produced by exposure and development, employing preferably the acid diamidophenol developer to conserve the blue print, which would be permanently reduced 40 to some extent in a strongly alkaline developer, but recovers nearly its original strength by simple washing in running water when the amidol developer has been employed.

Good results can be obtained with formulae considerably modified from that given,

but the formula given possesses the advantage that it substantially avoids a tendency to selective hardening of that part of the colloid containing the blue print, and leaves 55 the evenly distributed silver bromide content in the most favorable condition for the production of a perfect second image, which is another object of my invention.

The silver bromide layer after the above 60 treatment is somewhat less sensitive to light than it was originally, but quite sufficiently sensitive for my purpose.

Having thus described my invention, what I claim as new and desire to secure by 65 Letters Patent, is:—

1. The conversion of a photographic silver print in a colloid layer containing also silver bromide to a pigment blue print and silver bromide by treatment in a bath containing in combination the necessary ingredients for producing the blue image, and a bromide. 70

2. The conversion of a photographic silver print in a colloid layer containing also silver bromide to a pigment blue print and silver bromide by treatment in a bath containing in combination the necessary ingredients for producing the blue image, and a bromide, followed by exposure and development to produce a second image in the same 75 colloid layer.

3. The conversion of a photographic silver print in a colloid layer containing also silver bromide to a pigment blue print and silver bromide by treatment in a bath containing in combination the necessary ingredients for producing the blue image, and a bromide and a chloride. 85

4. The conversion of a photographic silver print in a colloid layer containing also silver bromide to a pigment blue print and silver bromide, by treatment in a bath containing in combination the necessary ingredients for producing the blue image, and a bromide and a chloride, followed by exposure and development to produce a second image in the same colloid layer. 90

FREDERIC EUGENE IVES

Witnesses:

H. S. FAIRBANKS,  
JOHN A. WIEDERSHEIM.